

Feb. 26, 1957

G. KATZ

2,783,208

POWDERED IRON MAGNETIC CORE MATERIALS

Filed Jan. 4, 1954



GRAMS 2,7 ISO-PROPYL NAPHTHALENE SODIUM  
SULFONATE PER 100 GRAMS POWDER

INVENTOR.  
*George Katz*

BY *J. L. Whittaker*  
ATTORNEY

2,783,208

## POWDERED IRON MAGNETIC CORE MATERIALS

George Katz, Philadelphia, Pa., assignor to Radio Corporation of America, a corporation of Delaware

Application January 4, 1954, Serial No. 401,767

7 Claims. (Cl. 252—62.5)

This invention relates to magnetic cores and more particularly to improved magnetic cores formed of compressed powdered iron.

Magnetic cores made of compressed powdered iron, the individual particles of which are insulated from each other and bound together by resinous materials are well known. They are generally suitable for use as induction cores to operate at relatively high electrical frequencies. One method of making such cores comprises mixing powdered iron with a dilute solution of a polybasic inorganic acid such as sulfuric or phosphoric acid. The iron is preferably, although not necessarily, prepared by the carbonyl process which produces relatively pure iron in the form of relatively small particles which may run about  $3\mu$ — $10\mu$  in size. In many instances it is important that the iron particles be of a small size since eddy current losses in a compressed core decrease as the particle size decreases.

Treating the powder with polybasic acid produces an insulating coating upon the individual iron particles. The powder is then mixed with a binder such as a phenol formaldehyde resin and molded into a desired shaped body.

One object of the instant invention is to provide an improved magnetic core.

Another object is to provide a compressed powdered iron magnetic core having improved electrical loss characteristics.

Another object is to provide a powdered iron magnetic core having improved physical strength and able to withstand relatively high stress.

Another object is to provide magnetic core bodies comprising powdered iron and having both improved strength and improved electrical loss characteristics.

These and other objects may be accomplished by the practice of the instant invention which provides an improved magnetic core body. It has now been discovered that improved core bodies may be produced by treating powdered iron with a polybasic acid solution that includes a relatively small proportion of a sulfonated derivative of naphthalene. The treated powder is molded according to previous practice to form core bodies of improved strength and having improved electrical properties.

The invention will be described in greater detail in connection with the drawing of which:

The single figure is a chart illustrating the improvement in properties provided by the practice of the instant invention.

According to a preferred embodiment of the instant invention a mass of carbonyl iron powder consisting essentially of iron particles about  $3\mu$ — $10\mu$  in their greatest dimensions is wet with a solvent such as acetone that does not react with iron. About 50—100 cc. of acetone are used for each 100 gm. of iron powder. For purposes of convenience the present example described the treatment of 100 gm. of powdered iron. Larger quantities

may be treated with correspondingly larger quantities of the other materials involved.

A second mixture is prepared by dispersing about .02 gm. of 2,7 iso-propyl naphthalene sodium sulfonate in about 50—100 cc. of the same solvent used to wet the iron, conveniently, acetone. About 1—5 gm. of granodine is added to the acetone-sulfonate solution. Granodine is a trade name for an aqueous 40% phosphoric acid solution that includes about 6%—12% by weight zinc phosphate.

The acetone-sulfonate-granodine mixture is added to the powdered iron and thoroughly mixed therewith. The mixture is continuously stirred and, preferably, is heated to a temperature of about 40°—50° C. to drive off substantially all the acetone and water. For small batches the mixing may be done in any convenient vessel such as a laboratory beaker. Larger quantities are preferably mixed in a mill such as a Simpson mixer. This treatment forms an insulating coating on the individual particles of the iron powder and prepares them for molding with a resin.

Any of a large number of phenol formaldehyde resins is satisfactory for molding core bodies according to the invention. A preferred resin is one that is known by the trade name of FD-4-80M (manufactured by the Acme Resin Corporation, 1401 Circle Avenue, Forest Park, Illinois). This product comprises a solution of about 60% phenol formaldehyde resin and 40% volatile solvent such as methyl alcohol. About 5 gm. of the resin solution is diluted with about 50—100 cc. of acetone. The treated iron powder is wet down with about 50—100 cc. of acetone and the diluted resin solution is added to the wet powder. The mixture is stirred continuously and gently heated to mix the resin and the iron powder intimately together and to drive off the acetone and moisture. This mixing may be conveniently carried out in a Simpson mixer or other mill to produce pellets of about 18—20 mesh average size.

A molding lubricant consisting of about  $\frac{1}{4}$  gm. of powdered zinc stearate or stearic acid is coated on the pellets by tumbling them in a barrel with the wax.

The pellets are then molded at about 50,000 lbs. per square inch pressure into bodies of a desired shape. The bodies are heated at about 145°—155° C. for  $\frac{1}{2}$  hour or more to cure the resin.

An essential feature of the invention is the inclusion of a sulfonated derivative of naphthalene in the granodine solution utilized in the initial treatment of the iron powder. The naphthalene derivative is preferably included in the granodine in the proportions of about .01—.08 gm. per 100 gm. of iron powder to be treated. The other steps heretofore described are not critical in the practice of the invention but may be varied within the general limits customary in the art. For example, powdered iron produced by processes other than the carbonyl process may be utilized and the particle size of the iron is not critical. Also, other polybasic inorganic acids such as sulfuric acid may be utilized in place of phosphoric acid. It is generally important, however, that the iron powder be relatively clean and free from grease and other organic matter.

Improved but somewhat less satisfactory results may be produced by substituting other sulfonated naphthalene derivatives in place of the iso-propyl naphthalene sodium sulfonate heretofore described. For example, an 18% improvement in transverse strength may be provided in a core body when utilizing the sodium salt of naphthalene-2,7 disulfonic acid in the proportion of about .04 gm. per 100 gm. iron powder. About a 10% improvement in strength is provided by 2-naphthalene sulfonic acid when utilized according to the invention in the proportions of about .01 gm. per 100 gm. iron powder. As may

be seen from curve B of the figure, however, a 38% improvement in transverse strength is provided by the use of 2,7 iso-propyl naphthalene sodium sulfonate as described heretofore in connection with the preferred embodiment.

It should also be noted that the practice of the instant invention provides a significant improvement in the electrical loss characteristics of a magnetic core. As may be seen from curve A of the drawing, "Q," an arbitrary inverse measure of electrical losses in a core body measured at 1 megacycle per second is improved about 4% by the practice of the preferred embodiment as described heretofore.

There have thus been described improved magnetic core bodies comprising powdered iron and a resin binder and also including relatively small proportions of a sulfonated naphthalene derivative. These bodies have improved strength and smaller electrical losses compared to previous bodies made in an exactly similar manner but without the sulfonated naphthalene derivative.

What is claimed is:

1. A method of making a compressed magnetic core body comprising the steps of wetting a mass of iron powder with a mixture comprising an aqueous solution of phosphoric acid and zinc phosphate and a substance selected from the group consisting of 2,7 iso-propyl naphthalene sodium sulfonate, the sodium salt of naphthalene 2,7 disulfonic acid, and 2-naphthalene sulfonic acid thereby, said substance being present in the proportions of about .01 to .08 gm. and said zinc phosphate being present in the proportion of about .06 to .60 gm. per 100 gms. of iron powder, to form an insulating coating upon the individual particles of said powder, drying said powder and molding said dried powder with a phenol formaldehyde resin binder to form a core body.

2. The method according to claim 1 in which said solution comprises 40% aqueous phosphoric acid and 6% to 12% by weight of zinc phosphate in acetone.
3. The method according to claim 2 in which said substance selected from said group is 2,7 iso-propyl naphthalene sodium sulfonate.
4. A product prepared according to the process of claim 1 wherein said substance is a sodium salt of naphthalene 2,7 disulfonic acid.
- 10 5. A product prepared according to the process of claim 1 wherein said substance is 2-naphthalene sulfonic acid.
- 15 6. A product prepared according to the process of claim 1 wherein said substance is 2,7 iso-propyl naphthalene sodium sulfonate.
7. The product of claim 6 wherein said 2,7 iso-propyl naphthalene sodium sulfonate is present in proportions of about .02 gm. per 100 gms. of iron powder.

20 **References Cited in the file of this patent**

UNITED STATES PATENTS

|           |                |               |
|-----------|----------------|---------------|
| 2,106,882 | Betz           | Feb. 1, 1938  |
| 2,227,945 | Neilson        | Jan. 7, 1941  |
| 2,306,198 | Verweij et al. | Dec. 22, 1942 |
| 2,601,212 | Polydoroff     | June 17, 1952 |

FOREIGN PATENTS

|         |               |               |
|---------|---------------|---------------|
| 403,373 | Great Britain | Dec. 15, 1933 |
| 523,864 | Great Britain | July 24, 1940 |

30 OTHER REFERENCES

Derkson, A. P. C. Spec. Serial No. 400,859, published April 27, 1943, 18-55M.